# EUROPEAN PATENT APPLICATION

(11) **EP 1 070 778 A1**
(43) Date of publication of application: **24.01.2001**
(21) Application number: 99870151.0
(22) Date of filing: 12.07.1999
(51) Int. Cl.: D04H 13/00, D05C 17/02

(54) **Method for the production of a reinforced non-woven material and products obtained with this method**

(71) Applicant: Wattex, 9255 Buggenhout (BE)
(72) Inventor: Baert, Paul, 1840 Londerzeel (BE)
(74) Representative: Pieraerts, Jacques

(57) **Abstract**

This invention relates to a method for the production of a reinforced nonwoven material based on stack fibres as a primary backing or tufted carpets, characterised in that the fleece is connected to filaments and/or threads.

## Description

The present invention relates to a method for the production of a reinforced non-woven material based on stack fibres as a primary backing for tufted carpets.

It is the aim of the present invention to produce a non-woven material as a primary backing for tufted carpets, using stack fibres which show a sufficient elasticity and strength to allow tufting and whereby the non-woven material is only partly damaged by the tufting needles.

Non-wovens in the way as they are currently used as primary backing in the carpet industry, were often produced using spun-bound fibres (i.e. endless filaments). The spun-bound fibres used thereby meet the following characteristics
■ they have a sufficient tensile strength in length and width direction (± 30 kg/5 cm);
■ an elongation at break of approximately 35%;
■ ensure a structure which allows an easy penetration of the tufting needles so as to damage the felt as little as possible.

To achieve this according to the invention, the fleece is connected to filaments and /or threads.

In a preferred embodiment of the invention, said filaments and/or threads are connected to the non-woven material through needling.

Still according to the invention the connection of the filaments and/or threads with the fleece can be performed through one of the following techniques: "stich bounding", water jets, glueing, or by making use of melting filaments and/or threads that are connected to the surface of the fleece by means of heat and pressure.

Other details and advantages of the invention will become clear from the following description of a method for the production of a reinforced non-woven material of this invention and of the products obtained with this method.

This description is given as an example and does not limit the invention.

To allow that the scope of the present invention be better distinguished from the state of the art, it should always be remembered that the non-woven materials that have been used up to now have always been produced with the so-called spun-bound technique. This means that the non-woven materials used as primary backing have always been made of endless filaments.

Spun-bounds uses thereto have an elongation at break of almost 30 kg/5 cm measured in length and width direction of the non-woven material. During the production of tufted carpets, it is necessary that the tufting needles can penetrate the non-woven material to a sufficient extent so as to damage the structure of the non-woven material as little as possible.

To provide a non-woven material suitable for use within the scope of the present invention, the fleece is made on the basis of stack fibres, and in fact by making use of one of the well known methods, in particular card or air-laid techniques. Preferably however use will be made of the card technique.

The stack fibres of which a fleece is built up are synthetic stack fibres or a mixture of synthetic and mineral and/or natural fibres. Also, as is moreover usual in the art, use can be made of melt and/or bicomponent fibres. In the latter case, the non-woven material can be integrally composed of such bicomponent fibres. A usual composition consists of a mixture consisting of 70% 3-den PES-filaments (with a length of 150 mm) and 30% of bicomponent fibres.

To ensure a sufficient tensile strength in the width direction, the stack fibres of the non-woven material are oriented in width direction as much as possible.

Since the major orientation of the fibres is to be found in width direction, the non-woven material can be needled in that way, so that the desired tensile strength as well as penetration possibility of the tufting needles is ensured.

The thus produced non-woven material has with respect to its weight, the desired tensile strength in width direction but in longitudinal direction however, this tensile strength is not ensured, According to the invention now, the tensile strength in longitudinal direction of the non-woven material is considerably increased by connecting filaments and/or threads with the fleece, at the surface of the fleece. An excellent technique through which filaments and/or threads can be connected to the surface of the fleece is needling. The needling presents the advantage that the threads and/or filaments are integrated into the non-woven material and in that way follow the movement of the non-woven material.

In case it is desired to further extend the "supporting function" of these filaments and/or threads, filaments and/or threads can also be needled to the surface of the fleece in width direction. By this support, these filaments and/or threads contribute to the conservation of the tensile strength and elasticity of the non-woven material, more precisely after the tufting needles have penetrated throughout the non-woven material. The filaments and/or threads used herein can be of synthetic as well as of mineral origin and it is also clear that use can be made of combinations of these filaments and/or threads. Also, use can be made of twinned filaments composed of synthetic filaments and/or mineral filaments and/or natural filaments.

It is clear that the desired tensile strength in longitudinal direction is determined by the number of filaments and/or threads that are applied to the surface of the fleece in this direction, through needling. A non-woven material that has been treated in this way has the desired tensile strength in length and width direction, but still has the high elasticity in both directions.

To obtain a fleece the elasticity of which meets the required standards, one of the following possible treatments can be applied:
a) thermal treatment
b) chemical/thermal binding.

When applying the thermal treatment mentioned under a) to the mixture that is used on the basis and consists of synthetic fibres and/or natural and/or mineral fibres, an amount of melting fibres and/or bicomponent fibres (preferably 25 to 30%). The basic material can also consist of 100% of bicomponent fibre or an amount of bicomponent fibre replenished with natural and/or mineral fibres. By exerting a suitable pressure, for example through the use of a calander or even more simple through the use of hot air, the melting fibres or the coat of bicomponent fibres are molten so that the other fibres within the mixture are mutually connected. The mutual connection between the different fibres of the non-woven material involves a decrease of the elasticity in length and width direction of the non-woven material.

When use is made of the method mentioned under b), the fibres of the mixture consisting of stack fibres, are glued to each other by means of a chemical binder (for example by means of a SBR or an acrylester). Through the application of hot air (± 200°C) the binder is dried and cured. This can be achieved by using a drying oven.

## Claims

1. A method for the production of a reinforced non-woven material based on stack fibres as a primary backing for tufted carpets, characterised in that the fleece is connected to filaments and/or threads.

2. A method as claimed in claim 1, characterised in that said filaments and/or threads are connected to the fleece through needling.

3. A method as claimed in claim 1, characterised in that said filaments and/or threads are connected through a technique known as "stich bounding".

4. A method as claimed in claim 1, characterised in that said filaments and/or threads are connected to the fleece by means of water jets.

5. A method as claimed in claim 1, characterised in that said filaments and/or threads are connected to the fleece through glueing.

6. A method as claimed in claim 1, characterised in that said filaments and/or threads are connected to the fleece by means of melting filaments and/or threads through the application of heat and pressure.
